# EUROPEAN PATENT SPECIFICATION

(11) **EP 0 846 199 B1**
(45) Date of publication and mention of the grant of the patent: **24.01.2001**
(21) Application number: 96928765.5
(22) Date of filing: 09.08.1996
(51) Int. Cl.: D21C 9/10, D21C 9/16

(54) **TREATMENT OF PULP WITH CHELATING AGENT IN AT LEAST TWO MIXING STEPS WITHOUT INTERMEDIATE WASHING**
ZELLSTOFFBEHANDLUNG MIT EINEM KOMPLEXBILDNER IN MINDESTENS ZWEI MISCHUNGSTUFEN OHNE ZWISCHENWÄSCHE
TRAITEMENT D'UNE PATE A PAPIER AVEC UN AGENT CHELATANT EN AU MOINS DEUX ETAPES DE MELANGE, SANS LAVAGE INTERMEDIAIRE

(30) Priority: 24.08.1995 SE 9502962
(43) Date of publication of application: 10.06.1998
(73) Proprietor: Valmet Fibertech Aktiebolag, S-851 94 Sundsvall (SE)
(72) Inventor: GERMGARD, Ulf, S-865 31 Alnö (SE); LINDQUIST, Jonas, S-856 41 Sundsvall (SE)
(74) Representative: Sundqvist, Hans
(86) International application number: SE9600996
(87) International publication number: WO9708380

(56) References cited:
- EP-A- 0 402 335
- WO-A-93/23607
- WO-A-94/29514
- WO-A-95/08666

## Description

This invention relates to the bleaching of chemical pulp with chlorine-free bleaching chemicals. The invention, more precisely, refers to the treatment of pulp by chelating agents in connection with the bleaching.
Totally chlorine-free bleaching (TCF) of chemical papermaking pulp has become a very great success, and the making of chlorine-free pulp in the world will soon have reached five million tons per year, which is a highly exceptional development considering that this bleaching method was introduced less than five years ago.
Bleaching is carried out in most cases by first treating the papermaking pulp to be bleached with a chelating agent of the type EDTA or DTPA. The chelating agent has the object to remove from the pulp certain metal ions, particularly manganese, copper, iron a.o. which would affect the bleaching result negatively if they remain in the pulp. The chelating agent step usually is designated by the letter Q.

After the Q-step the pulp is washed to eliminate the exposed metal ions from the pulp as completely as possible. Thereafter follows the bleaching, which normally is carried out with hydrogen peroxide, at times in combination with other bleaching steps and intermediate washing steps where ozone or peracids can be used. Hydrogen peroxide steps usually are designated by the letter P. According to a thumb rule, the more harmful metal ions are eliminated from the pulp in the Q-step, the more effective the subsequent bleaching will be.
A method, at which the pulp is treated in a Q-step and thereafter in a P-step,, usually is called the "Lignox"-method, as disclosed, for example, in EP-A-402 335.
The original pulp normally is oxygen delignified to a relatively low kappa number prior to the QP-bleaching. A low kappa number implies that the obtainable maximum brightness increases and the bleaching chemical demand decreases.
The QP-bleaching is carried out in mills most often in such a way, that the pulp first is passed through a pump, which pumps the pulp suspension through the treatment steps. Thereafter the chelating agent is admixed homogenously to the pulp in a mixer. The next step is a bleaching tower where the pulp without additional activation slowly passes through and where all remaining reaction takes place. The pulp finally is directed to a washing step where the exposed and complexed metal ions are washed out. The exposed liquid enriched on metal ions most often is discharged.
The conditions normally applied in a Q-step are a temperature of 70-90°C, a stay-time of 1-2 hours, a pulp concentration of 10-14%, a pH of 5-7 and a charge of chelating agent of 1-3 kg/ton pulp. The Q-step, from a strict bleaching point of view, actually is an unnecessary treatment step, because no increase in brightness takes place here. The Q-treatment, however, is necessary for a successful chlorine-free bleaching, as appears from above. If the Q-step could be simplified without thereby reducing the efficiency of metal elimination, great savings could be made, because a complete bleaching step with bleaching tower is expensive.
The present invention is directed to a solution of the aforesaid problems. By the invention, thus, the Q-step is made more efficient by eliminating the metals effectively at the same time as the Q-step is simplified, resulting in reduced investment costs in relation to a conventional Q-step.
The invention is based on the surprising discovery that the efficiency of the Q-step is affected considerably less by increased reaction temperature than by increased retention time. This indicates, according to classic chemical kinetics, that the Q-step is controlled by diffusion and not by reaction. The Q-step, consequently, should be carried out so that diffusion is facilitated. If this is done effectively, the total retention time can thereby be reduced considerably.

The characterizing features of the invention are apparent from the attached claims.

The best way of reducing the diffusion resistance is by decreasing the diffusion distance for active reactants and released reaction products.

This is achieved on technical scale by effective mixing, preferably in a mixer. The retention time in the Q-step, thus, can be reduced by repeated effective mixing. The number of mixing steps should be at least two, preferably at least three. For economic reasons, however, the number of mixing steps, and thereby the number of mixers, must be held on a reasonable level. A suitable number can be 2-4 steps. A certain retention time between the mixing steps is of good use, but this time need not be long, because the diffusion rate without mixing still is much slower than what is obtainable by mixing, for example in a mixer. The stay-time between the mixing steps, thus, shall be short, less than 15 minutes, suitably less than 10 minutes, and preferably less than 5 minutes. The mixing steps should be carried out one after the other, without intermediate washing. The washing required for removing the metals from the pulp suspension shall be carried out after the last mixing step.
The chelating agent preferably is of the type EDTA (ethylene diamine tetraacetic acid) or DTPA (diethylene triamine pentaacetic acid), but other types of chelating agent can be used, for example NTA (nitrilotriacetic acid) or DTPMP (diethylene triamine pentamethylene phosphonic acid). The total amount of added chelating agent should be 0,5-5 kg/t pulp (counted as pure chelating agent), preferably 1-3 kg/ t pulp.

The entire charge of chelating agent can be added in the first mixing step, whereby subsequent mixing steps bring about only repeated mixing. Alternatively, the chelating agent can be added in several of the mixing steps. The charging then should be made substantially in the first step, and in subsequent steps the added amount should be less than 2 kg/ t pulp per step.
The temperature in the mixing steps should be above 70°C and suitably above 80°C. A preferable temperature interval is 80-120°C.
The pressure in the entire Q-step preferably should be 1-10 bar.
An especially effective admixture can be achieved by uisng highly intensive mixers, which break-up the fiber network in the pulp and bring about close contact between fibers and chelating agent.
The invention, of course, is not restricted to the embodiments described above, but can be varied within the scope of the invention idea.

## Claims

1. A method for chlorine-free bleaching of pulp wherein metals are removed by means of a chelating agent, **characterized in** that the chelating agent is admixed to the pulp without use of a bleaching tower in at least two subsequent mixing steps without washing, that the stay-time between the mixing steps is less than 15 minutes, and that the pulp is washed after the last mixing step.

2. A method as defined in claim 1, **characterized in that** the entire charge of chelating agent is made in the first mixing step, whereby subsequent mixing steps bring about only repeated mixing.

3. A method as defined in claim 1, **characterized in** that the chelating agent is added in several mixing steps.

4. A method as defined in any one of the preceding claims, **characterized in** that the entire charge of chelating agent amounts to 0,5-5 kg/ton pulp, preferably 1-3 kg/ton pulp.

5. A method as defined in any one of the preceding claims, **characterized in** that the temperature in the mixing steps is above 70°C.

6. A method as defined in any one of the preceding claims, **characterized in** that the chelating agent is of the type EDTA or DTPA.

7. A method as defined in any one of the claims 1 - 5, **characterized in** that the chelating agent is of the type NTA or DTPMP.

8. A method as defined in any one of the preceding claims, **characterized in** that the admixing of the chelating agent is made by highly intensive mixers, which break up the fiber network in the pulp and bring about close contact between fibers and chelating agent.

9. A method as defined in any one of the preceding claims, **characterized in** that the mixing steps are carried out at a pressure of 1 - 10 bar.

## Patentansprüche

1. Verfahren zum chlorfreien Bleichen von Pulpe, wobei Metalle durch ein Chelatisierungsmittel entfernt werden,
**dadurch gekennzeichnet,**
daß das Chelatisierungsmittel der Pulpe beigemischt wird, ohne einen Bleichturm zu verwenden, in mindestens zwei aufeinanderfolgenden Mischstufen ohne Waschen, daß die Ruhezeit zwischen den Mischstufen weniger als 15 Minuten beträgt, und daß die Pulpe nach der letzten Mischstufe gewaschen wird.

2. Verfahren nach Anspruch 1,
dadurch gekennzeichnet, daß die gesamte Beschickung des Chelatisierungsmittels in der ersten Mischstufe erfolgt, wobei darauf folgende Mischstufen nur eine erneute Mischung mit sich bringen.

3. Verfahren nach Anspruch 1,
dadurch gekennzeichnet, daß das Chelatisierungsmittel in mehreren Mischstufen hinzugefügt wird.

4. Verfahren nach einem der vorhergehenden Ansprüche,
dadurch gekennzeichnet, daß die gesamte Beschickung des Chelatisierungsmittels 0,5 bis 5 kg/Tonne Pulpe beträgt, vorzugsweise 1 bis 3 kg/Tonne Pulpe.

5. Verfahren nach einem der vorhergehenden Ansprüche,
dadurch gekennzeichnet, daß die Temperatur in den Mischstufen höher als 70°C ist.

6. Verfahren nach einem der vorhergehenden Ansprüche,
dadurch gekennzeichnet,
daß das Chelatisierungsmittel zum Typ EDTA oder DTPA gehört.

7. Verfahren nach einem der Ansprüche 1 bis 5,
dadurch gekennzeichnet, daß das Chelatisierungsmittel zum Typ NTA oder DTPMP gehört.

8. Verfahren nach einem der vorhergehenden Ansprüche,
dadurch gekennzeichnet,
daß die Beimischung des Chelatisierungsmittels durch hochintensive Mischer erfolgt, die das Fasernetzwerk in der Pulpe aufbrechen und engen Kontakt zwischen Fasern und Chelatisierungsmittel herstellen.

9. Verfahren nach einem der vorhergehenden Ansprüche,
dadurch gekennzeichnet, daß die Mischstufen bei einem Druck von 1 bis 10 bar durchgeführt werden.

## Revendications

1. Procédé de blanchiment sans chlore d'une pâte à papier dans lequel les métaux sont éliminés au moyen d'un agent chélatant, caractérisé en ce que l'agent chélatant est mélangé à la pâte à papier sans utiliser une tour de blanchiment en, au moins, deux étapes de mélange consécutives sans lavage, en ce que le temps de séjour entre les étapes de mélange est inférieur à 15 minutes, et en ce que la pâte à papier est lavée après la dernière étape de mélange.

2. Procédé selon la revendication 1, caractérisé en ce que toute la charge d'agent chélatant est apportée dans la première étape de mélange, de sorte que les étapes de mélange consécutives entrainent seulement un mélange répété.

3. Procédé selon la revendication 1, caractérisé en ce que la charge d'agent chélatant est ajoutée en plusieurs étapes de mélange.

4. Procédé selon l'une quelconque des revendications précédentes, caractérisé en ce que toute la charge d'agent chélatant s'évalue entre 0,5 et 5 kg par tonne de pâte à papier, de préférence entre 1 et 3 kg par tonne de pâte.

5. Procédé selon l'une quelconque des revendications précédentes, caractérisé en ce que la température des étapes de mélange est de 70° C environ.

6. Procédé selon l'une quelconque des revendications précédentes, caractérisé en ce que l'agent chélatant est du type EDTA ou DTPA.

7. Procédé selon l'une quelconque des revendications 1 à 5, caractérisé en ce que l'agent chélatant est du type NTA ou DTPMP.

8. Procédé selon l'une quelconque des revendications précédentes, caractérisé en ce que le mélange de l'agent chélatant est effectué par des mélangeurs très puissants, qui cassent le réseau de fibres dans la pâte et entrainent un contact étroit entre les fibres et l'agent chélatant.

9. Procédé selon l'une quelconque des revendications précédentes, caractérisé en ce que les étapes de mélange sont réalisées sous une pression de 1 à 10 bars.
